

## UNITED STATES PATENT OFFICE

ROBERT E. RENO, JR., OF FOLLANSBEE, WEST VIRGINIA, ASSIGNOR TO FOLLANSBEE BROTHERS COMPANY, OF PITTSBURGH, PENNSYLVANIA, A CORPORATION OF PENNSYLVANIA

## METHOD OF PRODUCING LOW CORE LOSS MAGNETIC MATERIAL

No Drawing.

Application filed April 18, 1930. Serial No. 445,533.

My invention relates to the manufacture of steel sheets and primarily to a novel method of making, out of alloys of iron and silicon, sheets adapted to be used as laminæ for electrical apparatus having alternating magnetic fields, such for example as armatures for motors and generators, and particularly for transformer cores.

A particular object of my present invention is to produce a sheet which when associated with a plurality of similar sheets in electrical apparatus of the type indicated will exhibit a minimum core loss.

A further object is to provide sheets of the character indicated which will possess in addition to the electrical characteristics which form the primary object of the invention, desirable physical properties, such as an appreciable absence of brittleness, and a useful degree of hardness.

One preferred manner of practicing the invention will now be pointed out.

The material upon which my present process is, so far as I am aware, capable of being practiced with the best results, comprises alloys of iron and silicon in varying proportions, as follows:

For the armatures of relatively low powered motors, an alloy of commercially pure iron and .50 per cent silicon; for an improved grade of material for the same purpose, an alloy of commercially pure iron and 1.25 per cent silicon; for a still further improved grade of this material, an alloy of commercially pure iron and from 1.75 per cent to 2.25 per cent silicon; for a special dynamo material, an alloy of commercially pure iron and from 2.50 per cent to 3.50 per cent silicon; and for high wattage transformer cores of the highest grade, an alloy of commercially pure iron and from 3.75 per cent to 5.00 or more per cent silicon.

From the foregoing it will be apparent that my novel process hereinafter to be described may be practiced to advantage upon alloys of iron and silicon without regard to their specific analyses. I have found the process results in a decrease in core loss of from .71 to .67 watt per pound at 10,000 lines and 60 cycles, in terms of the Epstein test, on a

typical material analysis. Comparable reductions in core loss have been achieved by processing other analyses according to the principles of my novel method, so that it is to be understood that the exact proportions of iron and silicon in the material form no part of my present invention, and the claims hereinafter are not to be limited in their application to materials containing the alloy elements in any specific proportions.

By the term "commercially pure iron" I means ingot iron having the lowest commercially practicable proportions of the commonly inevitable impurities such as phosphorous, sulphur, manganese, carbon, and frequently a trace of copper.

In practicing my present method, commercially pure iron is made in any approved manner, as for example in an open hearth bath. The molten iron is tapped from the furnace into a ladle containing sufficient ferro-silicon to produce the analysis ultimately desired, according to the grade of sheet desired, as explained hereinabove.

The contents of the ladle are then teemed into molds and permitted to cool to solidity to produce an ingot.

The material for the sheets having been thus compounded, the manufacture of the sheets involves the following treatment: An ingot is first charged into a suitable reheat furnace and raised to about 2200 degrees F. The ingot is then reduced in cross section by forging, rolling, or in any other convenient manner, to form sheet bar stock. The dimensions of the sheet bar stock will obviously depend upon the dimensions of the sheets ultimately desired. A typical ultimate sheet dimension is 30×108 inches, with a thickness of 14 mils, and the invention will be exemplified hereinafter in terms of such ultimate sheet dimensions. Accordingly, in the example supposed, the sheet bar stock will be reduced to sections having a width of about 8 inches, a length of about 31½ inches, and a thickness of from  $\frac{3}{8}$  to  $\frac{7}{16}$  inch.

The sheet bars are next heated to bright red, or about 1600 or more degrees F., and passed transversely through hot rolls, for about three passes single, and one pass

matched, to elongate them to about 48 inches. It is to be understood that no specific number of passes is required in the practice of this step, the sole function of this rolling operation being to alter the dimensions of the material, to form the incomplete product known as a breakdown.

The breakdowns are conveniently matched in fours, and reheated to about 1500 degrees 10 F., at which heat they are given one or more passes through hot rolls, by which they are pulled to about 84 inch lengths. In this condition the sheets are known as runovers.

The runover pack of four sheets is then 15 doubled across its transverse axis to become eight sheets, 42 inches in length. The pack of eight sheets is then reheated to about 1500 degrees F. and given a sufficient number of passes through the rolls to attain a length 20 somewhat in excess of pattern length, i. e., about 115 inches, for a 108 inch sheet. It will be remembered that the sheets of the runover pack are about 31 $\frac{1}{2}$  inches wide.

The object of the steps in my process thus 25 far outlined is merely to reduce the ingot material to sheets approximating the ultimately desired dimensions. None of these preliminary steps is therefore essential to the practice of my invention, nor is the specific 30 combination of operations which I have used herein to exemplify a preferred embodiment of the invention necessary to the attainment of satisfactory results.

The next operation, however, I consider essential to the practice of my new process. This step consists in normalizing the sheets 35 of the pack, i. e., in treating the sheets to an anneal, including relatively slow cooling, in substantially the manner which will now be 40 described.

The pack of sheets is first sheared on two sides and its fish-tail end to a width of 30 inches, and a length slightly in excess of 108 inches, and then annealed, preferably by passage 45 through a suitable continuous annealing furnace. It is convenient, when the continuous annealing furnace is used, to pass the pack of sheets therethrough with its doubled end leading, to avoid the risk of having the relatively limp sheets sag down between the conveying disks or rolls of the furnace. The temperature of the annealing furnace, and the time of exposure of the sheets 50 therein, are so regulated that all the sheets 55 of the pack, including the innermost sheet, are raised to a temperature of 1450 degrees F. or higher. The passage of the pack through the annealing furnace is so regulated that the pack will leave the cooling 60 zone at a temperature of about 700 degrees F. I have found that this annealing step is effective in removing all strain from the hot rolling step and results in giving to the sheet a grain size characteristic of the particular 65 alloy when normalized.

Upon removal from the annealing furnace, the doubled end of the pack is sheared off, the pack is opened and pickled in any suitable pickling bath, such for example as sulphuric acid, to remove the scale on the sheets. The 70 sheets are then washed in water and dried.

The sheets are next given one or more passes through cold rolls merely to iron out surface inequalities and produce a truly flat sheet.

The sheets are next stacked in any convenient number on a cast steel annealing bottom, covered with a wrought or cast steel top, which is sealed against the bottom with sand. This box is then charged into a suitable annealing furnace, which is raised to a 80 temperature of approximately 1650 degrees F. or higher, and while in the annealing furnace an atmosphere of what is commercially known as carbo-hydrogen gas is circulated through the box. This gas is a mixture resulting from the cracking of natural gas and consists of approximately 88 per cent more or less of hydrogen and 12 per cent more or less of hydrocarbons. The gas is carbonized as well as reducing. The box with 90 its contents is kept in this condition for about nine hours or more. At the expiration of this time the box is allowed to cool in the furnace until its temperature has been reduced to about 800 degrees F. The manner of this cooling step I have found to be of importance, and I prefer to practice it by merely turning off the source of furnace heat so that the temperature of the sheets is lowered very slowly, and only by reason of the failure of the 100 heat supply; not by any positive quenching means.

When the temperature has cooled to about 800 degrees F. the box is drawn from the furnace and an atmosphere of natural gas is circulated through the box until the sheets have 105 cooled to about 300 degrees F.

When so cooled the sheets are removed from the box and the operation is complete.

It is to be understood that while I have 110 pointed out hereinabove one preferred manner in which the invention may be practiced, the description is merely by way of exemplification. Numerous variations in detail to suit individual preferences and the requirements of particular mills will readily suggest themselves to persons skilled in the art, but all such modifications, to the extent that they embody the principles of the invention as 115 pointed out in the appended claims, are to be considered within the scope and purview thereof.

What I claim and desire to secure by Letters Patent is:

1. The method of producing low core loss 125 magnetic material which consists in reducing an alloy of iron and silicon to a sheet, annealing the sheet in a continuous annealing furnace at a temperature of about 1450° F. or higher and removing the sheet from the 130

- cooling zone of the furnace at a temperature of about 700° F., then annealing for about nine hours at a temperature of about 1650° F. or higher in a carburizing and reducing atmosphere, then cooling the sheet in the furnace to a temperature of about 800° F. by removing the source of heat and then further cooling the sheet to about 300° F. in a reducing atmosphere. 70
- 10 2. The method as claimed in claim 1 including the steps of pickling and drying the sheet immediately after the first annealing step. 75
3. The method as claimed in claim 1 including the steps of pickling, drying, and cold rolling the sheet immediately after the first annealing step. 80
4. The method of producing low core loss magnetic material which consists in forming a sheet of an alloy of commercially pure iron and silicon, normalizing the sheet at an initial temperature of about 1450° F. and a final temperature of about 700° F., then annealing at a temperature of about 1650° F., and then slowly cooling the sheet. 85
- 25 5. The method of producing low core loss magnetic material which consists in forming a sheet of an alloy of iron and silicon, normalizing the sheet at an initial temperature of about 1450° F. and a final temperature of about 700° F., then annealing at a temperature of about 1650° F. or higher in the presence of a non-oxidizing gas, and then slowly cooling the sheet. 90
- 30 6. The method of producing low core loss magnetic material which consists in forming a sheet of an alloy of iron and silicon, normalizing the sheet at an initial temperature of about 1450° F. or higher and a final temperature of about 700° F., then subjecting the sheet while in the presence of a non-oxidizing gas to a heating influence to raise the sheet to a temperature of 1650° F. or higher, and then allowing the sheet to cool slowly by withdrawing the heating influence. 95
- 40 45 7. The method of producing low core loss magnetic material which consists in reducing an alloy containing iron and silicon to a sheet, heating the sheet to a temperature of 1450° F. or higher, slowly cooling to about 700° F., pickling, washing, then annealing at a temperature of 1650° F. or higher in a non-oxidizing and carburizing atmosphere, and then slowly cooling to about 800° F. 105
- 50 8. The method of producing low core loss magnetic material which consists in reducing an alloy containing iron and silicon to a sheet, removing strain from the sheet, pickling, washing, then annealing in a non-oxidizing and carburizing atmosphere by raising the sheet to approximately 1650° F. or higher, and then permitting the sheet to cool slowly. 110
- 55 9. The method of producing low core loss magnetic material which consists in reducing an alloy containing iron and silicon to a sheet, normalizing to remove from the sheet 115
- 60 10. The method of producing low core loss magnetic material which consists in reducing an alloy containing iron and silicon to a sheet, normalizing to remove from the sheet the strain of the sheet forming operations, pickling, washing, cold rolling, and then annealing by subjecting the sheet to a heating influence and then allowing the sheet to cool by slowly solely removing the source of heat. 70
- 65 11. The method of producing low core loss magnetic material which consists in reducing an alloy containing iron and silicon to a sheet, normalizing to remove from the sheet the strain of the sheet forming operations, pickling, washing, cold rolling, then annealing by subjecting the sheet to a heating influence to raise its temperature to approximately 1650° F. or higher, allowing the sheet to cool slowly to about 800° F. by removing the source of heat, and then cooling the sheet in a non-oxidizing atmosphere to about 300° F. 80
- 70 75 80 85 90 95 100 105 110 115 120 125 130
- In testimony whereof I affix my signature.
- ROBT. E. RENO, JR.

**CERTIFICATE OF CORRECTION.**

**Patent No. 1,869,078.**

**July 26, 1932.**

**ROBERT E. RENO, JR.**

**It is hereby certified that error appears in the printed specification of the above numbered patent requiring correction as follows: Page 2, lines 89 and 90, for "carbonized" read carburizing; and that the said Letters Patent should be read with this correction therein that the same may conform to the record of the case in the Patent Office.**

**Signed and sealed this 1st day of November, A. D. 1932.**

**(Seal)**

**M. J. Moore,  
Acting Commissioner of Patents.**